

(No Model.)

E. H. RUST.

MATERIAL FOR COVERING HEATED SURFACES.

No. 283,819.

Patented Aug. 28, 1883.



Witnesses.

John F. C. Toland  
Fred A. Powell.

Inventor

E. H. Rust.  
by Crosby & Gregory, Editors

# UNITED STATES PATENT OFFICE.

EPHRAIM HYDE RUST, OF BOSTON, MASSACHUSETTS.

## MATERIAL FOR COVERING HEATED SURFACES.

SPECIFICATION forming part of Letters Patent No. 283,819, dated August 28, 1883.

Application filed June 14, 1883. (No model.)

*To all whom it may concern:*

- Be it known that I, E. HYDE RUST, of Boston, county of Suffolk, State of Massachusetts, have invented an Improvement in Material for Covering Heated Surfaces, of which the following description, in connection with the accompanying drawing, is a specification, like letters on the drawing representing like parts.
- 10 This invention has for its object a novel compound or material for covering heated surfaces to prevent loss of heat by radiation. My novel material consists of infusorial earth, or, as it is called in Germany, where found, "infusorian erde," and paper-pulp—that is to say, that kind of pulp used in making paper.
- 15 The invention is shown in the accompanying sectional drawing as applied to a bit of steam-pipe.
- 20 The infusorial earth is a most excellent non-conductor; but when mixed and made plastic and applied to a heated surface it is apt to crack and scale off the said heated surface unless held together by some other substance.
- 25 As a binder for the infusorial earth I employ about twenty-five parts of pulp to seventy-five parts of infusorial earth, mixing the

same with a liquid, preferably water, until plastic, and, if desired, I may add lime or other cementitious material.

The pulp used will preferably be made from bagging or manila rope; but, instead, I may use a wood pulp with a fiber as long as possible.

The proportions above stated may be varied. The paper-pulp, besides acting as a binding material, also acts to prevent radiation. As a binder its fibrous nature adds largely to the cohesiveness of the covering, and being, when wet, very plastic, it admits of the covering being applied very evenly and thoroughly on all shapes of surfaces.

I am not the first to employ infusorial earth with a binder for covering heated surfaces.

I claim—

As a coating for heated surfaces, infusorial earth mixed with paper-pulp, substantially as described.

In testimony whereof I have signed my name to this specification in the presence of two subscribing witnesses.

EPHRAIM HYDE RUST.

Witnesses:

GEO. W. GREGORY,  
BERNICE J. NOYES.